

May 7, 1957

R. P. HEUER ET AL

2,791,116

REFRACTORY BRICK HAVING SPACER PLATES

Filed Aug. 19, 1953



INVENTORS.

Russell Pearce Heuer  
Mervin Adrian Fay  
By *Russell Pearce Heuer*

ATTORNEYS

1

2,791,116

## REFRACTORY BRICK HAVING SPACER PLATES

Russell Pearce Heuer, Bryn Mawr, and Mervin Adrian Fay, Narberth, Pa., assignors to General Refractories Company, Philadelphia, Pa., a corporation of Pennsylvania

Application August 19, 1953, Serial No. 375,094

6 Claims. (Cl. 72—35)

The present invention relates to refractory brick having unusually high resistance to spalling and particularly to such brick intended for use in suspended roofs or supported walls of furnaces.

The present application is a continuation-in-part of our copending U. S. application Serial No. 57,454, filed October 30, 1948, now Patent No. 2,652,793, for Refractory Brick Resistant to Spalling and Process.

A purpose of the invention is to increase the resistance of refractory brick against spalling at the hot face due to repeated changes in temperature, by creating a separate internal refractory cell bounded at the opposed sides by internal comolded oxidizable metallic plates.

Further purposes appear in the specification and in the claims.

In the drawings we have chosen to illustrate a few only of the numerous embodiments in which our invention appears, choosing the forms shown from the standpoints of convenience in illustration, satisfactory operation and clear demonstration of the principles involved.

Figure 1 is a perspective view illustrating a brick of the invention.

Figure 2 is a view similar to Figure 1 showing a modification.

In the drawings like numerals refer to like parts throughout.

Describing in illustration but not in limitation and referring to the drawings:

In the construction of many types of furnaces to be used at high temperature, such as open hearth steel furnaces, it is desirable to use suspended refractory brick and supported wall constructions. The refractories used for this purpose consist of the various basic refractories, of which the most widely used are magnesia, chrome-magnesia and magnesia-chrome. It is customary to lay the brick with oxidizable metallic spacers in the joints. Frequently such basic brick are used without previous kiln firing and in such cases the metallic spacers are desirably applied to the brick at the time of forming the brick.

In service of this character, failure of the refractory is primarily by spalling away of the brick at the hot end due to the temperature changes which the hottest part of the brick experience in the cycle of intermittent operation of the furnace. The changes in temperature cause the brick to expand and contract rapidly, and eventually the brick fracture and spall off along planes which are parallel to the exposed faces of the brick and located about one inch from the hot end. This spalling causes premature failure.

In a refractory roof or wall, each brick has its hot end exposed to the interior of the furnace, while the sides parallel to the major axis of the brick extend outwardly from the furnace interior and are protected from the heat by adjacent brick. The hot end may exhibit a temperature of 3000° F. at the time the finished heat of steel is tapped from an open hearth steel furnace. A

2

thermal gradient then prevails along the longitudinal axis of the brick.

After the furnace is tapped, the furnace doors are opened, the fuel is shut off and a large quantity of cold charge is placed in the furnace. As a result the hot end of the brick cools rapidly and its temperature may fall to 1000° F. Since the cooling is relatively rapid most of the temperature change is confined to the hot end of the brick, and at some interior point there is relatively little loss in temperature.

After charging of the furnace is completed, the fuel is again supplied to the furnace and the hot end of the brick rises in temperature until the gradient formerly existing is again established. This operating cycle is repeated again and again. The brick are thus subjected to repeated strains and finally fracture develops parallel to the hot end and the hot end spalls off. A new hot end is thus established, and this is subjected to similar treatment and gradually the brick are destroyed.

If we consider the brick as divided into elements parallel to the longitudinal axis and parallel to one another, it will be evident that the adherence of each element to its neighbor tends to set up tensile stresses across the hot face of the brick which tend to increase the thickness of the individual elements when the hot face cools rapidly during the furnace cycle. The tensile stress acting across the hot end may rise to a value which the refractory cannot stand, whereupon a crack will result at 90° to the hot end. The deformation of the elements of the brick may exceed the strain which the refractory is capable of standing and this will produce cracks parallel to the hot face.

On heating compressive forces are set up which produce deformation in the opposite direction from that caused by cooling.

We have observed that the presence of metallic spacers attached to the sides of the brick during forming of the brick minimizes the tendency of cracks to occur at the surface due to the strains set up by heating and cooling.

The exact nature of the action of the metallic spacers in preventing crack formation is not entirely clear. It is, however, evident that the spacers exert an effect in avoiding crack origin and propagation.

The spacers are usually made of ordinary low carbon steel, although they can be made of any oxidizable construction metal or alloy which will operate at the temperature of the hot end of the refractory. It will be evident of course that the spacers need not be oxidizable at room temperature so long as they oxidize at furnace temperature, and therefore stainless steel, such as the 18% chromium, 8% nickel grade or the 16% chromium grade or other alloys of iron and chromium may be used.

The heat of the furnace oxidizes the spacers at the hottest part of the brick and the iron or other metallic oxide formed reacts with the basic material present in the refractory, suitably magnesia or impurities in chromium ore. The resultant product welds together to form a monolithic structure which definitely resists crack formation.

Our studies indicate that the strain set up in the surface of the brick due to heating and cooling are greater if the transverse dimensions of the brick are greater.

We have discovered that improved resistance to spalling is obtained by imbedding in the brick at the time of molding, a plurality of oxidizable metallic spacer plates which are placed in a plane or planes parallel to the major axis of the brick and preferably approximately parallel to one of the faces of the brick which extends longitudinally in the furnace, thereby subdividing the brick into comolded cells of smaller dimensions, which can be heated and cooled with less strain at the outer surface. The

same mysterious action of the spacer plate which minimizes the crack formation when the plate is located at the edge of the brick likewise minimizes the crack formation at the edges of the cells within the brick. Therefore, spalling resistance is decreased due to a combination of the cellular effect on account of reduced dimensions subjected to strain, and the skin effect exerted by the oxidizable metallic spacer subdividing the cells.

While the partition wall between the cells should extend a major portion of the distance across the brick at the hot end (and most desirably at least  $\frac{3}{4}$  of each distance), it will be understood that there may be some remaining cross connection between the refractory where the partition does not fully extend across the brick. Likewise while the cell should run the major portion of the length of the brick, it will be understood that considerable benefit will be evident if the partition is located at the hot end and extends for a distance of even two or three inches from the hot end. Naturally for best results the cells should be separated for the major portion of the length of the brick beginning at the hot end.

The brick mix employed may, for example, be magnesia or refractory material high in magnesia, such as dead burned magnesite or electrically fused magnesia. It is important that the refractory material be of a basic nature, since certain refractories such as silica would react with the metallic spacers when they oxidize and would form fusible slags, destroying the roof. Chromite may be used instead of part of the material high in magnesia. For example mixtures of chromite with magnesia, containing for instance 75% of chromite and 25% of dead burned magnesite, may be used.

The amount of chromite present may be decreased for example to a composition containing 25% chromite and 75% of dead burned magnesite. Any other suitable basic refractory composition may be employed.

Bonding substances should preferably be added to secure bond without kiln firing. Organic binders such as sulphite pitch, dextrin, glue, gum arabic or inorganic binders such as water solutions of magnesium sulphate, magnesium chloride, sodium dichromate, sodium silicate and the like may be used. The amount of binder used should be sufficient to form a brick which is mechanically strong without kiln firing. Normally the binder will be of the order of one percent on the weight of the brick, and will seldom exceed two percent, and should never exceed five percent.

The pressure of molding the brick will in any case exceed 1000 pounds per square inch (70.3 kilograms per square centimeter), and preferably exceed 5000 pounds per square inch (351.5 kilograms per square centimeter) and will most desirably exceed 10,000 pounds per square inch (703 kilograms per square centimeter).

Where reference is made herein to a brick it is intended to include any standard refractory shape as well as any suitable block or shape provided with any suitable contour or attachment to engage a suitable hanger or support if any.

Figure 1 shows a brick 20 according to the invention, having refractory material 21 which is comolded with a suitably U-shaped metallic spacer plate 22 having a base of the U 23 which is on one longitudinal face of the brick and opposing arms of the U 24 and 25 which are on opposed longitudinally extending sides of the brick.

The arms extend desirably the full dimension or at least a major portion of the full dimension of the brick in the direction in which the arms extend away from the base of the U.

In order to interlock with the brick, projections or tongues 26 are lanced from the arms and extend inwardly and are comolded in the sides of the brick.

In the preferred embodiment the side of the brick opposite to the base of the U is provided with a preferably flat metallic plate 27, which preferably extends the full length of the face in the direction of the major axis of the

brick, although it will be understood that it may have suitable cutouts for a hanger opening or hanger projection if desired. Tongues or projections 28 are suitably lanced or otherwise formed from the spacer plate 27 and are embedded by comolding in the refractory.

Internal spacer plates or partition walls 30 of which two are shown in spaced relation extend in the direction from the base of the U 23 toward the opposing spacer plate 27 and are desirably secured to the base of the U as by spot welding at 31. The partition plates or internal plates 30 extend parallel to the sides of the U in the form shown, subdividing the brick in the particular embodiment into external refractory cells 32 and 33, beginning at or adjacent to the hot end 34, and internal refractory cell 35, likewise beginning at or adjacent to the hot end. The refractory cells formed are desirably equal.

It is not important for the purpose of the present invention whether or not the partition plates have tongues or interlocks comolded in the refractory similar to the 20 tongues or interlocks 26 and 28.

The partition plates will, where desired, extend the full length of the brick in the direction of the major axis as shown in Figure 1, but in some cases the partition plates 30' are shortened as shown in Figure 2, so that 25 room will be permitted for a hanger socket at the cold end of the brick.

It will be understood that the molding pressure in forming the brick is applied between the face of the brick located at the base of the U 23 and the plate 27 so that 30 the internal plates and the external plates are intimately associated with the refractory by comolding. Thus the internal plates extend across the major portion of the dimension of the brick in the direction of molding.

All of the plates comolded with brick are desirably 35 of oxidizable metal such as steel as already explained. The spacers and the partition plate are preferably of sheet or plate about  $\frac{1}{16}$  inch thick, although thicker or thinner spacers may be used. Spacers and partition plates thicker than  $\frac{1}{4}$  inch are not recommended because of the tendency of the metal to melt out rather than oxidize, and spacers thinner than  $\frac{1}{4}$  inch are not recommended because the oxidized layer formed is not adequately thick.

The molded brick are desirably dried for about 24 hours, after which they are ready for use without kiln 45 drying.

It will be evident that while the U-shaped plates will be preferred, flat plates on the external faces will sometimes be desirable.

In view of our invention and disclosure variations and 50 modifications to meet individual whim or particular need will doubtless become evident to others skilled in the art, to obtain all or part of the benefits of our invention without copying the brick shown, and we, therefore, claim 55 all such insofar as they fall within the reasonable spirit and scope of our claims.

Having thus described our invention what we claim as new and desire to secure by Letters Patent is:

1. A basic refractory brick composed of a refractory 60 of the class consisting of magnesia and mixtures of magnesia and chrome ore, said brick having generally parallel opposed outside longitudinal faces and a plurality of spaced oxidizable metallic plates extending in comolded relation longitudinally through the interior of the brick transverse to the intended hot face of the brick and over 65 a major cross section of the brick in substantially the same direction as said opposed outside faces, said oxidizable metallic plates dividing said refractory into outside and inside cells between said outside faces of the brick and said plates, and said plates being adapted to react 70 in the inside of the brick with the basic refractory and strengthen the refractory of said cells adjacent to said plates.

2. A basic refractory brick composed of a refractory 75 of the class consisting of magnesia and mixtures of magnesia and chrome ore, having external and internal

refractory cells, comolded external oxidizable metallic plates at opposed longitudinal outside faces of the brick, comolded internal oxidizable metallic plates interposed between said external and internal cells and extending through the interior adjacent to the hot face and extending over a major portion of the cross section of the brick, the external and internal plates being adapted to oxidize and the internal plates being adapted to react in the inside of the brick with the basic refractory and strengthen said external and internal cells.

3. A refractory brick of claim 2, further characterized in that the internal plates are generally parallel to the external plates.

4. A refractory brick of claim 2, in which the internal plates and the external plates are directly interconnected.

5. A refractory brick of claim 2, in which the internal cells and the external cells are of substantially equal size.

6. A basic refractory brick composed of a refractory of the class consisting of magnesia and mixtures of magnesia and chrome ore, said brick having generally parallel opposed outside faces, a plurality of spaced oxidizable metallic plates extending in comolded relation longitudinally through the interior of the brick transverse to the

intended hot face of the brick and over a major cross section of the brick in substantially the same direction as said opposed outside faces, and an oxidizable metallic plate extending in comolded relation over a longitudinal face of the brick other than said opposed outside longitudinal faces, and extending in a direction perpendicular to said internal plates, said oxidizable metallic internal plates dividing said refractory into outside and inside cells between said opposed outside faces of the brick and said 10 internal plates, and said internal plates being adapted to react in the inside of the brick with the basic refractory and strengthen the refractory of said cells adjacent to said internal plates.

15 **References Cited in the file of this patent**

UNITED STATES PATENTS

|           |        |                |
|-----------|--------|----------------|
| 2,247,376 | Heuer  | July 1, 1941   |
| 2,527,063 | Heuer  | Oct. 24, 1950  |
| 2,579,050 | Ramsay | Dec. 18, 1951  |
| 2,652,793 | Heuer  | Sept. 22, 1953 |
| 2,673,373 | Heuer  | Mar. 30, 1954  |